

96

Oct. 6, 1931.

A. E. SCHUTTE

1,826,529

METHOD OF FORMING CONCRETE STRUCTURAL UNITS

Filed May 16, 1929

Fig. 1



Fig. 2



Fig. 3

Inventor

August E. Schutte

By Dodge and Sons,

Attorneys

Patented Oct. 6, 1931

1,826,529

XR

## UNITED STATES PATENT OFFICE

AUGUST E. SCHUTTE, OF NORTHBORO, MASSACHUSETTS, ASSIGNOR TO WARREN BROTHERS COMPANY, A CORPORATION OF WEST VIRGINIA

## METHOD OF FORMING CONCRETE STRUCTURAL UNITS

Application filed May 16, 1929. Serial No. 363,506.

25-155

This invention relates to method of producing concrete structural units such as piles, retaining walls and the like, and particularly to such units where protection against the destructive action of sea water is essential.

In a copending application, Serial No. 259,981, filed March 7, 1928, which has become Patent No. 1,788,748, there is described the use of a protective coating consisting of hydraulic cement grout, agitated in a heated condition with asphalt. This coating is applied and allowed to set, after which it is heated to diffuse the asphalt which initially is in the form of dispersed nodules or particles.

The present invention is based on a somewhat similar procedure, effective to disperse asphalt throughout a concrete structural unit.

The invention will be described in connection with the accompanying drawings, in which:

Figure 1 is a view, partly in vertical section, of a wall or pile constructed according to my invention;

Figure 2 is a diagram illustrating the condition prior to diffusion of the asphalt by heating;

Figure 3 is a similar view after such diffusion.

There is prepared a batch of hydraulic cement concrete containing cement, sand, crushed stone (or gravel) and water. The components may be conveniently heated before mixing or the batch may be heated

during or after mixing, so that the temperature of the batch is at least as high as the melting temperature of the asphalt to be used. A suitable quality of asphalt, heated to about the same temperature is then added

to the concrete and mixed therewith by agitation until the asphalt is dispersed in fine nodules or particles uniformly throughout the mass. Changes in temperature and the duration of agitation affect the fineness of the dispersed asphalt particles and considerable latitude is permissible according to the final results desired.

The concrete thus formed is then allowed to set in forms. If the structural units to be produced are of uniform section, and not too

large ordinary practice is followed, but if the sections are irregular or large, so that uniform distribution of heat is impracticable without danger of differential heating and cracking one or more heat convector passages are formed in the unit and so spaced that the distribution of heat thereby will be substantially uniform throughout the unit.

In Figure 1 there is shown at 6 a passage of this character, extending axially through a pile 7. In the case of a wall or slab of similar thickness there would be a series of equally spaced parallel passages centered on the median plane of the wall.

After the concrete has set the asphalt will be found in fine dispersed nodules of particles 8 as illustrated in a somewhat exaggerated scale in Figures 1 and 2. After the concrete is set, the entire mass of the unit is heated by a medium applied externally and through the passages described (if any), the temperature being sufficient to fuse the asphalt nodules and to cause the same to diffuse through the porous structure of the dried concrete and to coalesce.

In Figure 3 there are illustrated a plurality of areas 9 in which the asphalt has diffused from the pockets in which the asphalt nodules were originally contained. The illustration is to an extent diagrammatic and is not precise.

Considerable latitude in proportions and in the order and degree of heating is contemplated.

What is claimed is:

1. The method of forming structural units which comprises, preparing an ordinary cement concrete containing aggregate, hydraulic cement and water; heating said concrete before it sets; heating asphalt; mixing the heated asphalt with the heated concrete and agitating the mixture until the asphalt is thoroughly dispersed in the form of fine masses; allowing the resulting mixture to set in the form of a structural unit; and finally heating said unit to cause the dispersed masses of asphalt to diffuse and coalesce.

2. The method of forming structural units which comprises preparing a heated batch of concrete containing aggregate, hydraulic ce-

ment, water and asphalt; agitating the same to ensure dispersion of the asphalt in small masses; allowing the concrete to set in the form of a structural unit having at least one core passage arranged to permit substantially uniform distribution of heating medium throughout the mass of said unit; and finally heating said unit by a heating medium distributed thereby and thus causing the dispersed masses of asphalt to diffuse and coalesce.

3. The method of forming structural units which comprises, preparing an ordinary cement concrete containing aggregate, hydraulic cement and water; heating said concrete before it sets; heating asphalt; mixing the heated asphalt with the heated concrete and agitating the mixture until the asphalt is thoroughly dispersed in the form of fine masses; allowing the resulting mixture to set in the form of a structural unit having at least one core passage arranged to permit substantially uniform distribution of heating medium throughout the mass of said unit; and finally heating said unit by a heating medium distributed thereby and thus causing the dispersed masses of asphalt to diffuse and coalesce.

In testimony whereof I have signed my name to this specification.

AUGUST E. SCHUTTE.